

1

3,506,410

**SYNTHESIS OF NEW URANIUM COMPOUNDS**  
Fritz Hulliger, Zurich, Switzerland, assignor to American Cyanamid Company, Stamford, Conn., a corporation of Maine  
No Drawing. Filed Apr. 9, 1968, Ser. No. 719,858  
Int. Cl. C01g 1/00

U.S. Cl. 23—346

10 Claims

## ABSTRACT OF THE DISCLOSURE

New uranium compounds of the formula UXZ, where X=S, Se, or Te and Z=P, As, Sb, or Bi. The compounds can be produced in large plate-like single crystals by the vapor transport method using the uranium halide UHal<sub>4</sub>, where Hal=Cl, Br, or I, or the halogens in elemental form. The compounds are ferromagnetic at low temperatures.

## BACKGROUND OF THE INVENTION

The general process of vapor transport, and particularly halogen vapor transport, is well known. However, as is in all vapor transport reactions, there is no single temperature range, the range depending on the nature of the products produced.

## SUMMARY OF THE INVENTION

The present invention is directed to new uranium compounds having the formula UXZ, in which X is S, Se, or Te, and Y=P, As, Sb, or Bi, preferably the compounds are formed as large plate-like single crystals.

The invention also includes a new process of making the compounds from their elements utilizing a modified halogen vapor transport, the transport gas being either elemental halogens Cl, Br, or I or uranium tetra-halide of the formula UHal<sub>4</sub>, where Hal can be any of the halogens above referred to. The process is very effective in the case of UPS, UPSe, UAaS, and UAaSe and particularly produces large single crystals.

It has been found that in the process modification of the present invention the high temperature zone is from 1000° to 1200° C., the other end of the transport vessel being from 50° to 100° C. cooler. Larger single crystals are produced in the cooler part with edge lengths up to 10 to 15 mm. and thicknesses ranging from about 0.2 to 1 mm.

The compounds of the present invention in their particular crystalline form are not limited to any single process of formation. Thus powders of mixed UXZ elements may be sintered separately before starting the halogen transport procedure or the elements may be used directly without preliminary sintering. In the latter case, the transport tube, which contains uranium turnings and pieces of the elements X and Z in stoichiometric ratio at one end together with the halogen transport gas or a uranium tetrahalide, is slowly heated to about 800° C. while avoiding a temperature gradient. The tube is kept at this temperature for some hours in order to permit formation of the desired compound in powder form. A temperature gradient is then produced having the gradient set out above.

The single crystals produced vary in color, for example white for USbTe, and have a metallic appearance. The crystal structure is of the same type as PbFCl, and when the crystals are colored they are usually brass colored. At room temperature the single crystals are paramagnetic but become ferromagnetic below about 100° K. Curie points vary somewhat from compound to compound.

It is an advantage that exact proportions of the reacting uranium and other compounds are not too critical. Ordinarily the uranium should be in a small excess because

2

having more uranium will merely speed up the reactions but will not change the nature of the compound produced. However, the ratio X:Z should be equal to one, since otherwise the UXZ crystals are intergrown with crystals of UX<sub>2</sub> or U<sub>3</sub>Y<sub>4</sub> or even UZ<sub>2</sub>. Excess arsenic and antimony may condense in elemental form. Usually the excess of uranium is very small and the ratio is substantially stoichiometric corresponding to 10<sup>-2</sup> to 3×10<sup>-2</sup> mole of UXY. In the case of UAaS the composition of the single crystals on checking by electron beam microanalysis was found to correspond exactly to the formula given.

The nature of the transport reaction is determined by the thermo-dynamic considerations of the reacting materials. In a great many cases the deposition of the transported material is at a cooler part of the equipment or transport path, and that is the case in the present reaction. This invention does not belong to the category represented, for example, by deposition of nickel with a carbon monoxide transport gas where the formation of the nickel carbonyl is at a lower temperature than its decomposition temperature at which metallic nickel is deposited. In the present case the temperatures are not very critical. As in a great many halogen vapor transport process, the temperature at one end of the transport path has to be quite high, frequently above 1000° C. In the present case it has been found that a very suitable temperature for the hot end of the transport zone is about 1000° to 1200° C., and the cooler portion where the large single crystals of the compound UXZ are deposited will be from 50° to 100° C. cooler. These temperatures are not critical and considerable variation can be present. This is a valuable, practical advantage of the process aspect of the present invention as it does not require extremely critical temperature control.

As in most halogen vapor transport processes, the concentration of the transporting vapor is comparatively small. In the present case a suitable desirable range is from 10<sup>-5</sup> to 10<sup>-4</sup> gram equivalents/cm.<sup>3</sup>, which corresponds to 1.3–13 mg. iodine/cm.<sup>3</sup>, 0.8 mg. bromine/cm.<sup>3</sup>, 0.35–3.5 mg. chlorine/cm.<sup>3</sup>. Again, this is not critical and the possibility of using the process without extremely critical control of this factor is a desirable feature.

In modification of the process starting from the elements themselves it is advantageous to cause them to react at lower temperatures, for example below 800° C., without any temperature gradient or even with a small gradient in the reverse direction. The temperature is not raised to the higher point of 1000° to 1200° C. until after the desired compound has formed. The other end of the transport vessel is kept 50 to 100° C. cooler.

As the compounds are new compounds, this aspect of the invention is not limited to any process and includes them regardless of the process by which they are formed. While it is possible to produce the compounds from powders, this presents some operating problems as uranium powder is neither easy to handle nor readily available. Therefore, it is preferred to use uranium turnings instead. This results in a smaller surface of uranium exposed to the reaction than would be the case with a powder, and so it takes a somewhat longer time to complete the reaction. Some speeding up of the reaction can be effected by shaking the reaction tube, which appears to remove layers of UXZ formed on the surface of the turnings. Alternatively, UXZ compounds may be prepared by sintering pressed mixtures of UX<sub>2</sub> and UZ<sub>2</sub> powders or UZ and X or UX and Z. The halogen vapor transport, however, is so efficient that the process feature is important and is included in a preferred modification of the invention. The crystals produced are single crystals and are quite large, for example 10 to 15 mm. edge length and from about 0.2 to 1 mm. thickness. Larger crystals are metallic in appearance and brass to white

colored as X, Z vary from light elements (S, Se, P, As) to heavier elements (Te, Sb, Bi) the brass color becomes more and more white. They have a crystal structure of the tetragonal PbFCl type and are semimetallic with resistivities of about  $10^{-4}$  ohm cm. at room temperature. As an example, the resistivity of UAsSe crystals has a value of  $5 \times 10^{-4}$  ohm cm. at 300° K. and a small but negative temperature coefficient between 100 and 700° K. The crystals are paramagnetic of the Curie-Weiss type. At a lower temperature the slope of the curve  $1/\chi$  vs. T becomes steeper and below about 100° K. the compounds are ferromagnetic. The exact point where the magnetic transition takes place will vary, of course, somewhat with the different compounds, as can be seen from the Table which follows the specific examples and summarizes data from them. For example, the compounds UAsS has a Curie point near 120° K. Since the crystals are tetragonal, their physical properties are anisotropic and they are useful for processes and equipment where these characteristics are desirable, particularly in the ferromagnetic range.

In the process aspect of the present invention it is an advantage that quartz tubes or quartz-lined tubes may be used. No coating with a protecting film is necessary at the temperatures used for UPS, UPSe, and UAsS and UAsSe, which is a further operating advantage. However, in the case of compounds which do not form easily, for example USbS, USbSe and USbTe, reaction with silica may prevent formation of the desired compound. Small single crystals of these compounds can be grown in carbon-coated quartz tubes.

#### DESCRIPTION OF THE PREFERRED EMBODIMENTS

The invention will be described in conjunction with the following specific examples.

##### Example 1

A slight excess of uranium turnings and pieces of arsenic and sulfur in amount corresponding to about  $2 \times 10^{-2}$  mole of the final UAsS compound are placed in one end of a closed quartz tube of 25–40 mm. diameter with a length of 200–250 mm. and a wall thickness of 1.5 to 2 mm. The tube is uncoated or may be carbon-coated on its inside. The quartz tube is evacuated, filled with chlorine gas in an amount of 2 mg./cm.<sup>3</sup> of the tube volume, and then closed. Alternatively chlorine may be introduced in the form of the requisite amount of UCl<sub>4</sub>. In the cases where Y is As, chlorine may be added as AsCl<sub>3</sub>.

The tube is slowly heated up to about 800° C., avoiding a temperature gradient, and is maintained at this temperature until equilibrium formation of the compound results. This can take approximately one day, but is not critical. Then the end of the quartz tube which contains the starting material is heated up to 1000°–1200° C. and the other end maintained 50° to 100° C. cooler. The transport tube may be tilted in order to accelerate flowing of the carrier

gas back to the hot end. Within one week single crystals of UAsS are formed in the cooler part of the tube. These crystals normally are square with edge lengths up to 5–10 mm. and a thickness of 0.2–0.5 mm.

After formation of the single crystals is substantially complete, the tube is slowly cooled down, opened, and the UAsS single crystals removed. Excess uranium and uranium tetrachloride may be recovered by conventional means and can be reused. The deposit consists of brass colored, metallic, plate-like crystals having a PbFCl structure with lattice constants as listed in the table. The crystals are paramagnetic at room temperature and become ferromagnetic below their Curie point of 120° K.

##### Example 2

The procedure is repeated with uranium tetrabromide or AsBr<sub>3</sub> or elemental Br. The same product is obtained, having the same crystalline and magnetic characteristics.

##### Example 3

The procedure of Example 1 is repeated, replacing the uranium tetrachloride with uranium tetraiodide or elemental iodine. The same products are obtained, and the transport is slightly faster with the iodine-containing transport gas. The crystals are also larger; edge lengths of 10–15 mm. and a thickness of 0.2–1 mm. are normal.

##### Example 4

The procedure of Example 3 was repeated, replacing the sulfur with selenium. Single crystals of UAsSe were produced and had similar physical characteristics, especially similar magnetic characteristics to the products of Example 3.

##### Example 5

The procedure of Example 3 was repeated, replacing the arsenic with a corresponding amount of phosphorus. The single crystals of UPS were produced and were similar in their chemical and physical characteristics, including magnetic characteristics, to those of Example 3.

##### Example 6

The procedure of Example 4 was repeated, replacing the arsenic with a corresponding amount of phosphorus. The crystals obtained of UPSe were similar in their chemical and physical characteristics, including magnetic characteristics, to the produce of Example 4. As in the case of all of the preceding examples, at low temperatures the crystals become ferromagnetic and are anisotropic.

##### Example 7

The procedure of Example 4 was repeated, replacing the selenium with a corresponding amount of tellurium. Single crystals of UAsTe were produced which, however, were smaller (up to 5 mm. edge length and 0.5 mm. thick) and almost white (only slightly brassy).

The characteristics of the different compounds, including lattice constants, are set forth in the following table:

| UXZ                | a(A.) $\pm 0.003$ | c(A.) $\pm 0.005$ | $\theta_f$ (° K.) | $\theta_p$ (° K.) | C <sub>M</sub>   | $\alpha$ ( $\mu\text{v}/^\circ\text{C}$ ) |
|--------------------|-------------------|-------------------|-------------------|-------------------|------------------|-------------------------------------------|
| UPS                | 3.813             | 7.981             | 120               | +70               | 0.53 (T>200° K.) |                                           |
| UAsS               | 3.874             | 8.158             | 120               | +110              | 0.55 (T>150° K.) | 25 (p)                                    |
| USbS <sup>1</sup>  | 3.937             | 8.530             | 150               | +140              | 0.68 (T>160° K.) |                                           |
| UPSe               | 3.961             | 8.178             | 90                | +60               | 0.69 (T>160° K.) | 2 (n)                                     |
| UAsSe              | 3.986             | 8.384             | 110               | +76               | 0.71 (T>180° K.) | 15 (p)                                    |
| USbSe              | 4.116             | 8.678             | 115               | +100              | 0.65 (T>180° K.) |                                           |
| UAsTe              | 4.167             | 8.764             | 100               | +78               | 0.77 (T>170° K.) |                                           |
| USbTe              | 4.321             | 9.063             | 110               | +100              | 1.0 (T>150° K.)  |                                           |
| UBiTe <sup>1</sup> | 4.434             | 9.157             | 110               |                   |                  |                                           |

a, c—Lattice constants of the tetragonal UXZ compounds.

$\theta_f$ —Ferromagnetic ordering temperature (Curie Point).<sup>2</sup>

$\theta_p$ —Paramagnetic Curie temperature (Weiss constant).<sup>2</sup>

$\alpha$ —Thermoelectric power near room temperature.

n, p—n- or p-type, respectively.

<sup>1</sup> Polycrystalline sample only.

<sup>2</sup> Derived from susceptibility measurements in the paramagnetic temperature range above the temperatures indicated in brackets according to the equation.

$$\chi_M = \frac{C_M}{T - \theta_p}$$

Where  $\chi_M$  = Suscept per mole.

It will be noted that the examples produce crystals of one cation only, but it is also possible to produce mixed crystals of UXZ and ThXZ as the two types of compounds have the same crystal structure. This has been verified in the case (U, Th)AsSe. However, in such a case when part of the uranium atoms are replaced a magnetic dilution results, that is to say, the magnetic moment per volume as well as the Curie temperature decrease.

I claim:

1. A compound UXZ in crystalline form in which X is selected from the group consisting of sulfur, selenium and tellurium, and Z is selected from the group consisting of phosphorus, arsenic, antimony and bismuth.

2. A compound according to claim 1 in the form of a plate-like single crystal, the crystal being metallic in appearance, white to brass colored, paramagnetic at room temperature, and ferromagnetic at temperatures below about 100° K.

3. As a new composition of matter crystalline UAsS.

4. A compound according to claim 3 in the form of a plate-like single crystal, brass colored, metallic in appearance, paramagnetic at room temperatures, being anisotropically ferromagnetic at temperatures below about 120° K.

5. As a new composition of matter crystalline UAsSe.

6. As a new composition of matter crystalline UPS.

7. As a new composition of matter crystalline UPSe.

8. As a new composition of matter crystalline USbSe.

9. As a new composition of matter crystalline USbTe.

5      10      15

10. A process of producing single crystals of a compound UXZ, in which X is selected from the group consisting of sulfur, selenium and tellurium, and Z is selected from the group consisting of phosphorus, arsenic, antimony and bismuth, by the halogen vapor transport system, which comprises subjecting U.X.Z powder mixture to reaction with a transport gas reaction atmosphere, where the transport gas is selected from the group consisting of chlorine, bromine and iodine, in a vapor phase transport equipment at a temperature of about 900°-1300° C. while maintaining another zone of the transport equipment from 50° to 100° C. cooler until large plate-like single crystals of the compound UXZ are produced in the cooler zone and recovering the crystals so produced.

#### References Cited

20      25

Norman, L. D., Thermoelectric Properties of Depleted Uranium Selenides and Tellurides, Bureau of Mines Report 6638, 1965.

Nuclor Science Abstracts 17-14856, Uranium Chalcogenides, May 15, 1963.

Nuclear Science Abstracts 17-24064, Nuclear Fuel Element Report, July 31, 1963.

CARL D. QUARFORTH, Primary Examiner

M. J. McGREAL, Assistant Examiner

UNITED STATES PATENT OFFICE  
CERTIFICATE OF CORRECTION

Patent No. 3,506,410

April 14, 1970

Fritz Hulliger

It is certified that error appears in the above identified patent and that said Letters Patent are hereby corrected as shown below:

Column 1, line 31, "YP" should read -- ZP --; line 39, "UAaS" should read -- UAsS --; same line 39, "UAaSe" should read -- UAsSe --. Column 2, line 5, "U<sub>3</sub>Y<sub>4</sub>" should read -- U<sub>3</sub>Z<sub>4</sub> --; line 39, after "0.8" insert -- -8 --.

Signed and sealed this 15th day of December 1970.

(SEAL)

Attest:

Edward M. Fletcher, Jr.

Attesting Officer

WILLIAM E. SCHUYLER, JR.

Commissioner of Patents